

## 1

3,318,700

**APPLICATION OF DYESTUFF BLEACHING CATALYSTS IN THE SILVER DYESTUFF BLEACHING PROCESS**

Walter Anderau, Aesch, Basel-Land, and Rudolf Mory, Dornach, Solothurn, Switzerland, assignors to Ciba Limited, Basel, Switzerland, a Swiss company

No Drawing. Filed Sept. 5, 1963, Ser. No. 306,690  
Claims priority, application Switzerland, Sept. 14, 1962,

10,928/62

16 Claims. (Cl. 96—53)

The silver dyestuff bleaching process for the production of color component images in photographic layers is based on the knowledge that certain organic dyestuffs, especially azo dyestuffs, are bleached out by photographically produced metallic silver, the degree of bleaching being dependent on the amount of silver present. Reduction of the azo groups occurs, which are split and converted into amino groups. In order to initiate this reaction, alkali-metal halides and other substances such as urea, thiosemicarbazide or especially thiourea or derivatives thereof generally must be present in the dyestuff bleaching bath in addition to acids such as hydrochloric acid, sulfuric acid or citric acid, examples of such alkali-metal halides being potassium bromide, potassium chloride and sodium chloride. A common silver dyestuff bleaching bath thus contains 30 to 80 parts of potassium bromide, 20 to 70 parts of thiourea and 35 to 70 parts of 30% sulfuric acid or hydrochloric acid in 1000 parts of water.

Although a wide choice is possible in respect of the proportions of the substances used, the bleaching time for different types of azo dyestuffs varies, for example, between 1 minute and 60 minutes. On the other hand, the gradation of the color image depends not only on that of the silver image but also on the bleaching time. If the silver dyestuff bleaching bath is allowed to act on the material for only a short period, the color image shows a flat gradation curve. The gradation curve becomes steeper the longer the dyestuff bleaching bath is allowed to act on the material. It has been observed that some azo dyestuffs are never quite fully bleached by the amount of silver normally present in a layer, the degree of bleaching achieved being at most to a density of 0.1 to 0.2 compared with the original logarithmic density of 1.0 to 2.0.

It has already been observed that certain substances substantially decrease the bleaching time, for example, from 20 minutes to 2 to 4 minutes, when added to the silver dyestuff bleaching bath in very small amounts. Moreover, dyestuffs that cannot be bleached at all or that cannot be fully bleached are completely bleached in the presence of such catalysts. Such catalysts are, for example, dimethyl-quinoxaline, pyridine, picolines, quinolines and aminothiazoles; especially effective are 2-hydroxy-3-aminophenazine and 2:3-diaminophenazine

(1)



(2)



The incorporation of a catalyst in the layer during the casting process together with the dyestuff has also been described.

## 2

The action of the catalysts on different types of azo dyestuffs varies considerably. It may be very effective with one kind of azo dyestuff and have virtually no catalytic effect on the bleaching process with another. Thus, there is a need for other catalytically active compounds which, either alone or in admixture with other catalysts, would make possible a uniform rate of bleaching for all three dyestuffs in multilayer material.

This invention is based on the observation that certain naphthazine compounds are especially suitable as dyestuff bleaching catalysts in the silver dyestuff bleaching process.

The present invention provides a process for the production of color photographic images by the silver dyestuff bleaching process wherein there is used an azine compound having at least one acidic group imparting solubility in water and corresponding to the formula

(3)



in which R<sub>1</sub> represents a naphthalene radical condensed with the azine ring in the manner indicated by the valence lines, which naphthalene radical carries a hydroxyl group, an amino group and/or an azo group attached to the six-membered ring not directly bound to the azine ring, and R<sub>2</sub> represents a benzene or naphthalene radical condensed with the azine ring in the manner indicated by the valence lines, as a dyestuff bleaching catalyst.

The compounds of the Formula 3 contain at least one acidic group imparting solubility in water, for example, a sulfonic acid or a carboxylic acid group. Such groups can be bound directly to the carbon atoms which are ring members of the azine compounds, but carboxylic acid groups, in particular, can also be joined to the carbon atoms of the ring systems R<sub>1</sub> and/or R<sub>2</sub> through a bridge member, for example, through a —CH<sub>2</sub>— or an —O—CH<sub>2</sub>— group.

The naphthalene radical R<sub>1</sub> is condensed with the azine ring in such a manner that two adjacent carbon atoms of the naphthalene ring, advantageously in  $\alpha$ : $\beta$ -position, are shared with the azine ring. The naphthalene radical R<sub>1</sub> contains a hydroxyl group or an amino group or an azo group attached to the six-membered ring not directly bound to the azine ring; it can also contain more than one of these groups, for example, a hydroxyl group and an amino group or a hydroxyl group and an azo group. A sulfonic acid group can also be present in this ring. The azo group which is bound on one side to the naphthalene radical R<sub>1</sub> is bound on the other side, for example, to a benzene radical or to another naphthalene radical.

R<sub>2</sub> can be a benzene radical or a naphthalene radical, which can also correspond to the definition of R<sub>1</sub>, thus forming, for example, azine compounds having a centrosymmetric constitution of the kind exemplified by Formula 6a.

The radicals R<sub>1</sub> and R<sub>2</sub> and more especially the radicals bound to the naphthalene radicals through an azo group can contain further substituents of the kind defined or other substituents, for example, halogen atoms such as chlorine, alkyl groups such as methyl and ethyl groups and alkoxy groups such as methoxy and ethoxy groups. Even larger molecules of azine compounds of the Formula 3 can be built up, for example, by reacting aminoazo compounds of this kind with phosgene or cyanuric chloride to form urea or triazine compounds.

Specially important are the azine compounds containing at least one sulfonic acid group that correspond to the formula

(4)



in which R<sub>2</sub> has the meaning given above and R<sub>4</sub> represents an amino group or an azo group bound to a further aromatic radical. Also worthy of special mention are the azine compounds of the formula

(5)



(in which R<sub>2</sub> and R<sub>4</sub> have the meanings given above), and also those of the formula

(6a)



or

(6b)



in which R<sub>4</sub> and R'<sub>4</sub> may be identical or different and represent an amino group or an azo group bound to a further aromatic radical.

Some of the azine compounds to be used in the process of the invention are known; the azine compounds can be prepared by known methods.

In the process of the invention the said catalysts may be added to the dyestuff bleaching bath in a solution containing one gram of catalyst per liter of water in an amount of 1 to 50 cc. per liter of bleaching bath. In a bath that contains for example, 30 parts of potassium bromide, 30 parts of thiourea and 35 parts of 30% hydrochloric acid in 1000 parts of water, a blue azo dyestuff of the formula

(7)



for example, is bleached very slowly, and even after 30 minutes the layer is not quite colorless at the places where the silver was at maximum density, but if a solution of 1 g./liter of the catalyst of the formula

5

(8)



15

is added to such a bleaching bath in an amount of 1 to 4 cc. per liter of bleaching bath, other conditions being the same, the places where the silver was at maximum density are completely colorless after 3 to 6 minutes. Similar 20 results are obtained with the catalysts of the formulae

25



30

and

(10)



35

40

45

50

55

60

65

The catalysts herein described can be used singly, in pairs or in mixtures comprising more than two such catalysts and, if desired or required, they can also be used in admixture with other catalysts, for example, pyridine, aminohydroxyphenazine or quinoxaline. It is also possible to allow the catalysts to act on the material for some minutes in a separate bath prior to the treatment in the bleaching bath. If this procedure be adopted the material can be treated in the subsequent silver dyestuff bleaching bath without a catalyst of the invention or in the presence of other catalysts. Finally, it is also possible to add the catalysts to the emulsion prior to casting, thus incorporating them in the layer along with the silver halide and the dyestuff. By adopting this method, it is possible to incorporate in each dyestuff gelatine layer of three-color material the catalyst most suitable for each individual layer thus making possible a uniform bleaching of all the layers within the same period of time.

5

The non-diffusing naphthazine compounds of the following formulae are specially suitable for incorporation in the layers:

6

$m$ =an integer of at least 6  
 $n=1$  or  $2$

The compound of the Formula 15 contains a diffusion inhibiting substituent in the radical of the diazo com-



ponent (I). Compounds also suitable for use as catalysts in the process of the present invention are those of the formulae

(16)



75

7

(17)



An advantage of the catalysts to be used is that they are only slightly oxidizable.

The preparation of some of the azine compounds whose compositions are given above are described in the following:

The azine compound of the formula

(18)



0.5 mol of 1-aminobenzene-4-sulfonic acid is diazotized in the usual manner, and the diazo suspension is mixed with 0.5 mol of 2-phenylamino-5-hydroxynaphthalene-7-sulfonic acid and 500 cc. of water, while cooling with ice. The pH value of the coupling mixture is then adjusted to 2.5 to 3.0 by the addition of sodium acetate. The mixture is stirred for 3 hours at 0 to 5° C. and then for 16 hours at room temperature. Concentrated hydrochloric acid is then added until the pH value is 0.8 to 1.0 and the mixture is heated for 1 hour at 80 to 90° C. The temperature is allowed to drop to about 50° C., whereupon the mixture is filtered and the filter radical is washed with 5% hydrochloric acid. The product so obtained of the Formula 16 is then pasted in 1/2 liter of water, and the pH of the mixture adjusted to 7 by the addition of sodium hydroxide solution and sodium acetate. The mixture is quickly suction-filtered, and the filter radical recrystallized from water. The yield is about 75% of the theoretical yield. The product is a green-yellow powder when dry.

By using in the place of 2-phenylamino-5-hydroxynaphthalene-7-sulfonic acid an equivalent proportion of 2-(4'-methoxyphenyl)-amino-5-hydroxynaphthalene-7-sulfonic acid, 10-methoxy-4-hydroxybenzo[a]phenazine-2-sulfonic acid of the formula

15 is obtained by the same process. It is a yellow-olive powder.

0.1 mol of 4-hydroxybenzo[a]phenazine-2-sulfonic acid of the Formula 16 are introduced into 500 cc. of water. A diazo suspension prepared in the usual manner from 0.1 mol of 1-aminobenzene-4-sulfonic acid is added thereto. The pH value is adjusted to 9.8 to 10.0 by the subsequent addition of sodium carbonate, and the coupling mixture is stirred for 16 hours at room temperature. The dyestuff is then precipitated with sodium acetate and filtered. It is then dissolved in 1200 cc. of water, the solution is adjusted to pH 7.5 with a small amount of acetic acid, and the dyestuff is again precipitated with sodium acetate. The dyestuff is again isolated by filtration, washed free from acetate with ethyl alcohol and dried in vacuo at 50° C. The yield is about 85% of the theoretical yield. The azine compound of the Formula 18 so obtained is a dark brown powder. The aminoazine compound of the Formula 17 can be obtained from this azine compound containing an azo group by reduction with sodium hydrosulfite.

By coupling diazotized aromatic monamines or tetrazotized diamines with the hydroxyphenazines of the Formulae 8, 16 and 19, further azoazines are obtained that can be used as dyestuff bleaching catalysts. These products are prepared by known methods, for example, by the method used to prepare the substance of the Formula 18 described above.

As examples of products that can be prepared in this manner there may be mentioned those of the Formulae 12 and 13, and those of the following formulae

(20)



(21)



(22)



(23)



(24)



The following table indicates the color of these substances in a neutral aqueous solution, in an aqueous sodium hydroxide solution and in an aqueous hydrochloric acid solution.

TABLE I

| Formula number | Color in—        |                        |                           |
|----------------|------------------|------------------------|---------------------------|
|                | H <sub>2</sub> O | NaOH                   | HCl                       |
| (12) -----     | Brown-red        | Violet                 | Bordeaux <sup>1</sup>     |
| (13) -----     | Yellow-brown     | Grey-blue              | Red-brown <sup>1</sup>    |
| (20) -----     | do               | Red-brown <sup>1</sup> | Yellow-brown <sup>1</sup> |
| (21) -----     | Bordeaux         | Blue                   | Grey-blue <sup>1</sup>    |
| (22) -----     | Dull orange      | Dull orange            | Brownish                  |
| (23) -----     | Red-violet       | Grey-blue              | Grey-blue                 |
| (24) -----     | Red              | Bordeaux               | Violet                    |

55

60

The following examples illustrate the invention, the parts being by weight unless otherwise stated:

#### Example 1

The following layers are applied successively to a cellulose acetate film provided with an adhesive layer:

(1) A red-sensitized silver bromide emulsion in gelatine that contains the cyan dyestuff of the formula

(25)



<sup>1</sup> Precipitation.

(2) Gelatine intermediate layer.

(3) A green-sensitized silver bromide emulsion in gelatine that contains the magenta dyestuff of the formula



(4) A yellow filter layer that contains the dyestuff of the formula



(5) A blue-sensitized silver bromide emulsion in gelatine that contains the dyestuff of the formula

25 in an amount that gives an R-density of 0.75 is applied to a cellulose acetate film provided with an adhesive



and as precipitating agent a mixture comprising the reaction product of dicyano-diamidine and formaldehyde, a small amount of sodium formate and sodium bisulfate.

(6) A gelatine protective layer.

This film is exposed four times behind a neutral wedge in the following manner:

(1) With red light only,

(2) With green light only,

(3) With blue light only,

(4) With red, green and blue light,

the exposure being controlled in such a manner that the fourth wedge appears a neutral grey after processing.

After hardening in a formaldehyde bath, the film is developed in a Metol-hydroquinone developer and then treated in an acetic acid stop bath and in a fixing bath containing thiosulfate.

After washing in water for about 5 minutes, the film is treated in the following dyestuff bleaching bath:

|                                                                                                    |       |            |      |
|----------------------------------------------------------------------------------------------------|-------|------------|------|
| Potassium bromide                                                                                  | ----- | grams      | 100  |
| Thiourea                                                                                           | ----- | do         | 10   |
| Hydrochloric acid (37%)                                                                            | ----- | cc         | 70   |
| 1.25% solution of the addition product of 35 mols of ethylene oxide and 1 mol of octadecyl alcohol | ----- | cc         | 10   |
| Azine compound of the Formula 18                                                                   | ----- | milligrams | 3    |
| Bulked with water to                                                                               | ----- | cc         | 1000 |

The film is then washed with water, the residual silver is re-halogenated in a copper sulfate or copper nitrate bath made strongly acid with hydrochloric acid, washed again, fixed for the second time, washed and then dried. The time of treatment in the dyestuff bleaching bath should be just sufficient to bring about complete bleaching of the dyestuffs in all layers at the places most highly exposed, the said time of treatment having been determined by tests. It is much shorter than when the operation is carried out without the phenazine compound in the dyestuff bleaching bath.

12  
Example 2

A silver bromide gelatine emulsion that contains the cyan dyestuff of the formula

| Catalyst, formula No. | Amount of catalyst, mg./liter | Time of treatment in pre-treatment bath, min. | Time of treatment in dyestuff bleaching bath, min. |
|-----------------------|-------------------------------|-----------------------------------------------|----------------------------------------------------|
| 12                    | 10                            | 10                                            | 5                                                  |
| 13                    | 50                            | 10                                            | 5                                                  |
| 16                    | 10                            | 5                                             | 3                                                  |
| 17                    | 10                            | 5                                             | 3                                                  |
| 19                    | 10                            | 5                                             | 3                                                  |
| 20                    | 50                            | 10                                            | 5                                                  |
| 21                    | 10                            | 10                                            | 6                                                  |
| 22                    | 50                            | 10                                            | 5                                                  |
| 23                    | 50                            | 10                                            | 5                                                  |
| 24                    | 50                            | 10                                            | 5                                                  |

70  
Example 3

A colored gelatin silver bromide layer is prepared by mixing 5 grams of 5% aqueous solution of a cyan dyestuff of the formula

(30)



15

with 3.3 grams of a silver bromide gelatine, casting 10 cc. of this mixture on to a glass plate measuring 13 cm. x 18 cm. and then drying it. The layer so prepared is exposed under a master image and the silver image is developed in a developer that contains 6 grams of 1-methylamino-4-hydroxybenzene, 6 parts of anhydrous sodium carbonate, 20 parts of sodium borate and 80 parts of crystalline sodium sulfite per liter of water. After a short rinse, the layer is fixed for 5 to 7 minutes 20 and bleached in a silver dyestuff bleaching bath that contains 30 to 70 cc. of 37% hydrochloric acid, 20 grams of potassium bromide, 20 to 50 grams of thiourea and 4 cc. of an 0.1 aqueous solution of the catalyst of the Formula 8 per liter of water. After bleaching for 8 to 10 minutes at 20 to 22° C., the dyestuff is bleached at the areas containing silver to a degree proportional to the amount of silver present. After removal of the excess silver in a bleach fixing bath, a color image is obtained the dark and light areas of which exhibit the same blue tint. By 30 using instead of the azine compound of the Formula 8, 2-hydroxy-3-aminophenazine of the Formula 1 as catalyst or dimethyl-quinoxaline, the tint of the areas of the image that are only partly bleached is changed to red-violet and the image is therefore unusable. The silver halide layer described herein can form a part of three-color material.

*Example 4*

A solution of 5 mg. of the dyestuff of the Formula 29, 40 20 mg. of 2-phenylamino-4:6-dichloro-1:3:5-triazine-4'-sulfonic acid and 0.1 mg. of the catalyst of the Formula 12 in 3.5 cc. of water is mixed with 3.3 cc. of 6% gelatine solution and 3.3 cc. of silver bromide gelatine. The mixture is cast on a glass plate measuring 45 13 cm. x 18 cm. provided with an adhesive layer. When the layer is dry it is exposed in the usual manner behind stepped wedges and the silver image developed and fixed in the usual manner.

When a color silver image prepared in the above manner is treated for 5 to 10 minutes in a bleaching bath of the same composition as that given in Example 2, a blue stepped wedge that is bleached pure white at the areas where the original density of silver was greatest was obtained after removal of the residual silver and fixation.

When exactly the same procedure is followed, but with the catalyst omitted, almost no perceptible bleaching of the cyan dyestuff occurs, even after a treatment of 15 to 20 minutes in the bleaching bath.

What is claimed is:

1. A process for the production of a color photographic image by the silver dyestuff bleaching process, which comprises carrying out the bleaching operation in the presence of an azine catalyst that contains at least one acidic group imparting solubility in water and that corresponds to the formula



in which R<sub>1</sub> represents a naphthalene radical condensed with the azine ring in the manner indicated by the valence lines which naphthalene radical contains at least one sub-

stituent selected from the groups consisting of a hydroxyl group, an amino group and an azo group, said substituent being attached to the six-membered ring not directly bound to the azine ring, and R<sub>2</sub> represents a member selected from the group consisting of a benzene radical and a naphthalene radical condensed with the azine ring in the manner indicated by the valence lines.

2. A process for the production of a color photographic image by the silver dyestuff bleaching process, which comprises carrying out the bleaching operation in the presence of an azine catalyst that contains at least one sulfonic acid group and that corresponds to the formula



in which R<sub>2</sub> represents a member selected from the group consisting of a benzene radical and a naphthalene radical condensed with the azine ring in the manner indicated by the valence lines, and R<sub>4</sub> represents a member selected from the group consisting of an amino group and an azo group bound to a further aromatic radical.

3. A process for the production of a color photographic image by the silver dyestuff bleaching process, which comprises carrying out the bleaching operation in the presence of an azine catalyst of the formula



in which R<sub>2</sub> represents a benzene radical condensed with the azine ring in the manner indicated by the valence lines, and R<sub>4</sub> represents an amino group.

4. A process for the production of a color photographic image by the silver dyestuff bleaching process, which comprises carrying out the bleaching operation in the presence of an azine catalyst of the formula



in which R<sub>2</sub> represents a naphthalene radical condensed with the azine ring in the manner indicated by the valence lines, and R<sub>4</sub> represents an amino group.

5. A process for the production of a color photographic image by the silver dyestuff bleaching process, which

15

comprises carrying out the bleaching operation in the presence of an azine catalyst of the formula



5

10

in which R<sub>2</sub> represents a benzene radical condensed with the azine ring in the manner indicated by the valence lines, and R<sub>4</sub> represents an azo group bound to a benzene radical.

6. A process for the production of a color photographic image by the silver dyestuff bleaching process, which comprises carrying out the bleaching operation in the presence of the azine catalyst of the formula



20

25

7. A process for the production of a color photographic image by the silver dyestuff bleaching process, which comprises carrying out the bleaching operation in the presence of the azine catalyst of the formula

16



10. A process for the production of a color photographic image by the silver dyestuff bleaching process, which comprises carrying out the bleaching operation in the presence of the azine catalyst of the formula



30

11. A process for the production of a color photographic image by the silver dyestuff bleaching process,



8. A process for the production of a color photographic image by the silver dyestuff bleaching process, which comprises carrying out the bleaching operation in the presence of the azine catalyst of the formula

which comprises carrying out the bleaching operation in the presence of the azine catalyst of the formula



60

65

70

9. A process for the production of a color photographic image by the silver dyestuff bleaching process, which comprises carrying out the bleaching operation in the presence of the azine catalyst of the formula



12. A process for the production of a color photographic image by the silver dyestuff bleaching process, which comprises carrying out the bleaching operation in the presence of the azine catalyst of the formula



13. A process for the production of a color photographic image by the silver dyestuff bleaching process, which comprises carrying out the bleaching operation in the presence of the azine catalyst of the formula 15



14. A process for the production of a color photographic image by the silver dyestuff bleaching process, which comprises carrying out the bleaching operation in the presence of the azine catalyst of the formula



15. A process for the production of a color photographic image by the silver dyestuff bleaching process, which comprises carrying out the bleaching operation in the presence of the azine catalyst of the formula



19

16 A process for the production of a color photographic image by the silver dyestuff bleaching process,

20

which comprises carrying out the bleaching operation in the presence of the azine catalyst of the formula



**References Cited by the Examiner**

**UNITED STATES PATENTS**

2,410,025 10/1946 Gaspar ----- 96-53  
 2,627,461 2/1953 Friedman ----- 96-53

J. TRAVIS BROWN, *Primary Examiner.*

NORMAN G. TORCHIN, *Assistant Examiner.*

UNITED STATES PATENT OFFICE  
CERTIFICATE OF CORRECTION

Patent No. 3,318,700

May 9, 1967

Walter Anderau et al.

It is hereby certified that error appears in the above numbered patent requiring correction and that the said Letters Patent should read as corrected below.

Column 15, lines 3 to 12, for the right-hand portion of the formula reading "R<sub>3</sub>" read -- R<sub>2</sub> --.

Signed and sealed this 21st day of November 1967.

(SEAL)

Attest:

Edward M. Fletcher, Jr.

Attesting Officer

EDWARD J. BRENNER

Commissioner of Patents